

## UNITED STATES PATENT OFFICE

2,138,599

## CONTACT ELEMENT

Childress B. Gwyn, Jr., Bannockburn, Ill., assignor to P. R. Mallory & Co., Inc., Indianapolis, Ind., a corporation of Delaware

No Drawing. Application July 14, 1937,  
Serial No. 153,639

4 Claims. (Cl. 206—166)

This invention relates to electrical make and break contacts.

An object of the invention is to provide an electrical make and break contact which is suitable for use in connection with magnetos, relays and similar devices.

Another object is to provide an electrical make and break which may be substituted for contacts of the platinum, iridium and similar types.

10 A further object is the provision of an electrical make and break contact of comparatively high hardness and which, compared to contacts commonly used in the various fields mentioned, is relatively free from carburization.

15 Other objects of the invention will be apparent from the following description taken in connection with the appended claims.

The present invention comprises the combination of elements, methods of manufacture, and 20 the product thereof brought out and exemplified in the disclosure hereinafter set forth, the scope of the invention being indicated in the appended claims.

While a preferred embodiment of the invention is described herein, it is contemplated that 25 considerable variation may be made in the method of procedure and the combination of elements without departing from the spirit of the invention.

30 For many purposes, such as for magneto contacts, relay contacts, etc., it has heretofore been customary to use electrical make and break contacts composed of platinum-ruthenium or platinum-iridium alloys. While such contacts are 35 fairly satisfactory due to their hardness and non-corrosiveness in normal and most industrial atmospheres, a low transfer (carry-over) under the electric arcing inherent to magneto and most relay operations, they possess the disadvantages of high initial cost and difficulty of fabrication. 40 Moreover, the alloys platinum and iridium have shown a marked affinity for hydro-carbon vapors under electrical arcing conditions and this characteristic seems to increase with the increased 45 percentages of iridium necessary to produce sufficient mechanical strength and hardness of magneto and similar uses.

According to my invention an electrical contact is formed of an alloy of silver with palladium 50 or platinum, nickel and copper. It is preferred that the ingredients be present in the following ranges of proportions:

|                                   | Per cent |
|-----------------------------------|----------|
| Silver                            | 50 to 80 |
| Palladium or platinum             | 12 to 25 |
| Copper                            | 5 to 15  |
| Nickel—in excess of a trace up to | 7        |

55 In place of nickel I may substitute an element 60 having the alloying characteristics of this metal

It will be noted that this alloy contains a predominance of silver. This alloy is well suited for substitution for platinum or palladium base alloys in the fabrication of electric contacts.

As examples of specific contact alloys which have been found especially suitable after exhaustive life tests and actual service operation the following two compositions are representative:

| Contact alloy A |          | 10 |
|-----------------|----------|----|
|                 | Per cent |    |
| Silver          | 60       |    |
| Palladium       | 23       |    |
| Copper          | 12       |    |
| Nickel          | 5        | 15 |

| Contact alloy B |          | Per cent |
|-----------------|----------|----------|
|                 | Per cent |          |
| Silver          | 67       |          |
| Palladium       | 14       | 20       |
| Copper          | 13.4     |          |
| Nickel          | 5.6      |          |

The contact in this invention compares favorably in the electrical characteristics with platinum or palladium base contacts, particularly on relay and magneto service, and is superior to such contacts from a carburization standpoint when exposed to hydrocarbon vapors. As compared 25 with palladium base or platinum base contacts there is, in addition to other advantages, a substantial saving in cost.

The contacts have also been found to be well suited for thermostatic control contacts and for contacts to work in atmospheres which are normally destructive to contacts, such as in gases containing  $H_2S$ ,  $SO_2$  or  $NH_4OH$ . They are also useful wherever a very light contact pressure must be used, or a current of low value must be used, even at extremely high rates of operation. 30 40

The density of the alloy is comparatively low so that the cost per contact is low.

This alloy can be substituted for white gold, and can be used in jewelry, for a thermostatic material, for pyrometer controls and for dental 45 inserts as well as for electrical contacts.

Contacts may be formed of the alloy by any of the usual methods of fabrication, such as by upsetting or heading, by screw machine operations, by molding or stamping or other methods.

This contact material has a relatively low vapor pressure, and consequently does not arc heavily or transfer readily when used on direct or pulsating current and, therefore has a low 55 co-efficient of contact resistance rise.

It shows little or no tendency toward oxidation in service.

While the present invention as to its objects and advantages, has been described herein as 60

carried out in specific embodiments thereof, it is not desired to be limited thereby but it is intended to cover the invention broadly within the spirit and scope of the appended claims.

5. What is claimed is:

1. An electric contact element formed of an alloy composed of about 5 to 15% copper, in excess of a trace up to 7% nickel, 12 to 25% of an element selected from the group consisting of 10 palladium and platinum and 50 to 80% silver.
2. An electric contact element formed of an

alloy composed of about 12% copper, 5% nickel, 25% palladium and 60% silver.

3. An electric contact element formed of an alloy composed of about 13.4% copper, 5.6% nickel, 14% palladium and 67% silver.

4. An electric contact element formed of a preponderance of silver and containing 5 to 15% copper, 12 to 25% of an element of the palladium-platinum group and in excess of a trace up to 7% nickel.

CHILDRESS B. GWYN, JR.